

Patented July 15, 1924.

1,501,336

# UNITED STATES PATENT OFFICE.

FRANZ HASSSLER, OF HAMBURG, GERMANY, ASSIGNOR, BY MESNE ASSIGNMENTS, TO THE CHEMICAL FOUNDATION, INC., A CORPORATION OF DELAWARE.

## TANNING.

No Drawing.

Application filed September 24, 1917. Serial No. 192,925.

To all whom it may concern:

Be it known that I, FRANZ HASSSLER, citizen of the State of Hamburg, Germany, residing at Hamburg, Germany, have invented new and useful Improvements in Tanning, of which the following is a specification.

I have found that I can convert hides into valuable leather by treating them with 10 heat-condensation products of aromatic sulfonic acids which are free from hydroxyl groups other than those occurring in sulfonic acid residues such as can be obtained by simply heating the sulfonic acids. Condensation products of this kind, especially 15 those derived from aromatic hydrocarbons, have strong tanning properties, even if the sulfonic acid of the hydrocarbon itself has but weak or no tanning efficiency, as is the 20 case with naphthalene, or toluene, sulfonic acids. As an instance of suitable condensation products which serve for the purpose of the present invention I mention the products obtained by heating sulfonic acids of 25 naphthalene (alpha or beta), methyl naphthalene, anthracene, toluene, or mixed sulfonic acids of toluene and naphthalene, or of derivatives of hydrocarbons, which are free from hydroxyl groups other than those 30 occurring in sulfonic acid residues, such as carbazol sulfonic acids, all of which condensation products are easily soluble in water and strongly precipitate glue solutions.

The following example sets forth an illustrative method by means of which bodies of the above-mentioned type may be prepared, said method being presented more in detail in my co-pending application Serial No. 192,923, filed September 24, 1917.

40 Equal parts of naphthalene and concentrated sulphuric acid are heated for about 8 hours at 130° C. The temperature is then raised to 170° or 180° C., and the heating is continued until, upon diluting 45 the reaction mixture with water, complete solution of the reaction products takes place.

The product, when cold, is a solid, glass-like mass, which is readily soluble in water and capable, in acid solution, of precipitating gelatine or glue from solutions of the same.

The process of tanning with the aid of 50 the aforesaid sulfonic acids can be carried 55 out in the usual way, but attention is to be

called to the fact that the said substances have a strongly acid character and I prefer to employ them in a nearly neutralized condition and to keep the bath in a moderate acid state by adding, if required, small 60 quantities of an acid. The said substances can also be employed together with natural tanning materials. In most cases a very fair leather is produced and even if dark colored natural tanning materials are employed, the leather can often be cleared up by simultaneously or afterwards treating with the aforesaid sulfonic acids. Thus, the heat-condensation product derived from naphthalene sulfonic acids produces a 70 white, or but slightly colored leather, whilst the condensation product obtained by heating anthracene sulfonic acid tans hides while simultaneously producing a thoroughly dyed full black shade.

Hides, skins and the like may be tanned with the products hereinbefore mentioned in the following manner:

Take for example 100 lbs. of hides, skins and the like which have been limed and bated, place said hides in a drum and treat at ordinary temperature with a slightly acid aqueous solution of a density of about 30° Bé. of a condensation product obtained as above outlined, such as a condensation product of a naphthalene sulfonic acid and maintain the acidity of the bath by additions of small amounts of dilute sulfuric acid. After about six to eight days, the tanning is complete, whereupon the 90 hides are removed and dried, subsequent to which they may, if so desired, be greased and finished in the usual manner.

Having now fully described my invention, what I claim is:

1. The process of tanning hide which consists in treating the hides with a slightly acid aqueous solution containing a water-soluble glue-precipitating heat-condensation product of an aromatic sulfonic acid, 100 said heat condensation product being free from methylene groups and free from hydroxyl groups other than those occurring in sulfonic acid residues.

2. The process of tanning hides which 105 consists in treating the hides with a slightly acid aqueous solution containing a water-soluble glue-precipitating heat-condensation product of a sulfonic acid of an aromatic hydrocarbon, said heat-condensa-

tion product being free from methylene groups and free from hydroxyl groups other than those occurring in sulfonic acid residues.

5 3. The process of tanning hides which consists in treating the hides with a slightly acid aqueous solution containing a water-soluble glue-precipitating heat-condensation product of naphthalene sulfonic acid, said 10 heat-condensation product being free from methylene groups and free from hydroxyl groups other than those occurring in sulfonic acid residues.

4. The process of tanning hides which 15 consists in treating the hides with a slightly

acid aqueous solution containing a water-soluble glue-precipitating heat-condensation product of naphthalene sulfonic acid, said heat-condensation product being free from methylene groups and free from 20 hydroxyl groups other than those occurring in sulfonic acid residues, and said product being obtained by treating naphthalene with concentrated sulfuric acid at 130° C. for 8 hours, raising the temperature to 25 170°-180° C., and heating until the product is completely soluble in water.

In testimony whereof I have hereunto set my hand.

FRANZ HASSLER.